

# UNITED STATES PATENT OFFICE.

CHARLES R. GOSTLING, OF EUSTIS, FLORIDA.

## METHOD FOR TREATING STEEL AND IRON IN THEIR MANUFACTURE.

1,091,330.

Specification of Letters Patent. Patented Mar. 24, 1914.

No Drawing.

Application filed June 12, 1913. Serial No. 773,310.

To all whom it may concern:

Be it known that I, CHARLES R. GOSTLING, a citizen of the United States, residing at Eustis, in the county of Lake, State of Florida, have invented certain new and useful Improvements in Methods for Treating Steel and Iron in Their Manufacture; and I do hereby declare the following to be a full, clear, and exact description of the invention, such as will enable others skilled in the art to which it appertains to make and use the same.

This invention relates to an improved method of treating steel and iron in the manufacture thereof.

In producing steel and iron it frequently happens that the product is of a low grade owing to the presence of an excess of gases, piping and blow holes, the ingot being unclean and when same is rolled the product does not possess the requisite tensile strength, ductility and clear surface.

It is therefore the object of the present invention to provide an improved method of treating steel and iron in its manufacture whereby all gases will be drawn from the product, piping prevented, and the presence of blow holes eliminated so that when the product is rolled it will possess maximum tensile strength, ductility, and a clear surface.

In carrying the invention into practice I place a quantity of diatomite or infusorial earth sometimes known as Kieselguhr in a mold, ladle or furnace and then fill same with the molten steel or iron it is desired to treat, after which I place a quantity of diatomite or infusorial earth upon the top of the molten steel or iron. The steel or iron delivered to the mold or ladle and engaged with infusorial earth or diatomite in the manner referred to will remain in a molten state much longer than under ordinary conditions of casting an ingot. As a result of the steel remaining in a molten state over a prolonged period the gases contained therein will have ample time to escape and such

escape of the gases is accelerated by the absorbent qualities of the diatomite or infusorial earth. In this way the ingot will be completely cleared and rendered free from piping and blow holes. The steel or iron thus treated will possess, when rolled, great tensile strength and ductility together with an absolutely clear surface. The reason for the diatomite or infusorial earth maintaining the steel in a molten state over a prolonged period is not known at this time but actual practice has proven such to be the case. It will be noted that as the molten steel or iron is poured into the ladle the diatomite in the bottom of the ladle rises upon the top of the molten mass but does not pass through the same. In this way the diatomite forms a blanket which protects the molten mass from the atmosphere during the operation of pouring and as a result the temperature of the mass during the operation of pouring is lowered very little owing to the blanketing action of the diatomite.

What I claim is:—

The herein described method of treating steel and iron in its manufacture consisting of placing a quantity of diatomite or infusorial earth upon the bottom of a receptacle, filling said receptacle with molten steel or iron and entirely covering the exposed face of the molten steel or iron with a quantity of diatomite or infusorial earth, and thereby maintaining the steel or iron in a molten state beyond the normal time required for solidification to allow the escape of all gases from the molten mass under the influence of the tendency of such gases to rise and expand, and under the influence of the absorbent qualities of the diatomite or infusorial earth.

In testimony whereof, I affix my signature, in the presence of two witnesses.

CHARLES R. GOSTLING.

Witnesses:

T. STEN HASELTON,  
W. M. SIMMONS.